

March 28, 1961

YUN JEN

2,977,245

SURFACES OF DECREASED WATER WETTABILITY  
AND PROCESS FOR THE PREPARATION THEREOF  
Filed June 24, 1957



INVENTOR.  
YUN JEN

BY

*Evan Kahn*

ATTORNEY

1

2,977,245

## SURFACES OF DECREASED WATER WETTABILITY AND PROCESS FOR THE PREPARATION THEREOF

Yun Jen, Stamford, Conn., assignor to American Cyanamid Company, New York, N.Y., a corporation of Maine

Filed June 24, 1957, Ser. No. 667,700

19 Claims. (Cl. 117—72)

The present invention relates to a process for treating hydrophilic surfaces to decrease their wettability by water and to the novel surfaces thereby produced.

It is known that hydrophilic surfaces may be rendered water-repellent by contacting the surfaces with a dilute aqueous solution of certain long chain aliphatic amine salts such as octadecylamine hydrochloride so as to form an amine coating thereover, as disclosed in U.S. Patent No. 2,356,542, granted to C. K. Sloan on August 22, 1944. According to the patent the amines form a coating over the hydrophilic surfaces causing them to become hydrophobic. The process of the patent has two major disadvantages.

(1) The coating is non-durable in that it is substantially completely removed when the treated surface is washed with soap and water.

(2) The water-repellence is fugitive in that the effect largely disappears within a few months.

The discovery has now been made that hydrophilic surfaces can be treated to decrease their wettability by water by a process which comprises two principal steps. In the first step, the surface is contacted with a dilute aqueous solution of a cationic high molecular weight amine polymer as hereinafter more particularly described, whereby at least some of the polyamine is irreversibly adsorbed by the surface. In the second step, the surface is contacted with sufficient of a dilute aqueous solution of a soap having a hydrophobic anion to convert at least some of the adsorbed polyamine to hydrophobic soap form. Thereafter the surface may be dried. By this process it is readily feasible to form sufficient hydrophobic polyamine soap on the surface to render the surface strongly water-repellent, as if oiled. Surprisingly, the bond between the adsorbed hydrophobic polyamine soap and the surface is so strong that polyamine soap is removed only to a negligible extent when the surface is flushed with water. Even more surprisingly, washing with soap and water generally increases the water repellence of the surface.

In the process, the amount of water-repellence developed and the luster of the surfaces are improved by flushing the surface with plain water after each treatment so as to remove any unadsorbed polyamine which may be present before the surface is contacted with the dilute aqueous soap solution and to remove any excess soap solution before the surface is allowed to dry.

From the foregoing it will be seen that the product of the present invention is a surface which is rendered water-repellent by the presence thereon of irreversibly adsorbed hydrophobic polyamine soap. Our evidence indicates that maximum water-repellence is achieved when the polyamine soap is present in amount approximately equivalent to a monomolecular layer. However, the invention includes surfaces on which a substantially smaller amount of polyamine soap is present.

The invention does not depend upon the particular surface treated. Very satisfactory results have been obtained in the case of Portland cement, glass and brick;

2

vitreous enamel; wood; paper; cotton cloth; hydrophilic baked organic enamel; hydrophilic nitrocellulose lacquer; and leather.

Articles which it is desired to make water-repellent 5 may be treated by complete immersion in either or both of the treating solutions or by brushing, spraying or rolling therewith. In most instances, only sufficient contact time with the polyamine solution is needed to cause at least some of the polyamine to be adsorbed as base 10 for the soap, and in the case of the second step for at least some of the adsorbed polyamine to be converted to hydrophobic soap form. Longer contact times give greater water-repellence, best results being obtained when the hydrophilic surface is contacted with polyamine solution until the adsorptive capacity therefor is substantially satisfied and when the application of soap solution is continued until formation of polyamine soap substantially ceases. Both steps proceed rapidly, and in practice, there is little advantage in allowing more than about 5 20 minutes for either. Very satisfactory results have been obtained with contact times of less than one minute.

The polyamines employed in the present invention have average molecular weights in excess of about 10,000. When the molecular weight of the polymer is 25 materially less, the water-repellence imparted by the treatment is fugitive, the coating being more or less readily washed away and being subject to absorption into the substrate with passage of time. Furthermore, the polyamines contain at least one amino nitrogen atom 30 having at least one ionizable or replaceable hydrogen atom for every 10 carbon atoms in the molecule, as it is through such atoms that the molecule as a whole is anchored to the substrate and to which the hydrophobic soap anions are attached. Substantially better results 35 are obtained when this ratio is increased to 1:5 and better results still when the ratio is increased to 1:2 as in the case of polyethylenimine or polyvinylamine.

The invention does not depend upon the concentration of either the polyamine or the soap in the two treating solutions employed. Satisfactory results have been obtained when both have been employed at concentrations as low as 0.01% and the evidence is thus that more dilute solutions yield useful results. The invention does not depend upon the adsorption of any particular amount of polyamine during treatment. The evidence is that not even a complete monomolecular layer is needed to provide sufficient polyamine as base for at least a significant amount of soaps. In particular instances optimum conditions of treatment are conveniently found by trial as illustrated in the examples.

The polyamine solutions appear to be most advantageously applied at about neutrality (pH 6-8) but good results have been obtained over the range pH 4-10. The soap solutions are likewise advantageously applied at about neutrality and in general may be applied within 55 the pH range in which they are stable.

A large number of synthetic polyamine condensation products are known which can be used as primary treating agents in the process of the present invention. They 60 may be essentially linear as in the case of the carbon-nitrogen chains formed by homopolymerization of ethylenimine or C-methylethylenimine. Similar materials may be prepared by condensing an alkylendiamine with an alkylenedichloride. Preferably the alkylendiamine and alkylenedichloride are selected so that the total number 65 of the linear chain carbon atoms included by the diamine groups of the alkylendiamine plus the linear chain carbon included by the chlorine atoms of the alkylenedichloride is between about 5 and 9 inclusive. Useful products thus may be prepared by condensing 1,2-propanediamine with 1,3-dichloropropane wherein the total number 70 of included carbon atoms is 5, or by condensing



employed were siliceous (glass, concrete, brick), cellulosic (cotton shirting and paper), and lignin (wood).

Each sample was treated by immersion (with occasional gentle agitation) for five minutes at room temperature in a 0.1% aqueous solution of polyamine agents adjusted to pH 9.0, after which the sample was rinsed for five minutes under a stream of fresh water to remove any unadsorbed polyamine present. The sample was then immersed for five minutes in at least 20 times its weight of 0.1% aqueous sodium stearate solution at room temperature, rinsed again, and allowed to dry at room temperature.

The samples were tested by tilting to an angle of 45° and allowing a slow stream of water to flow thereover for about a minute. During the test the tendency of the droplets (into which the stream broke) to adhere to the surface was noted. A rating of 1 was given to denote substantially complete water-repellence with substantially no wetting (as if the surface had been oiled). A rating of 2 was given to denote good initial water repellence with development of slight subsequent wetting, and a rating of 3 to denote a substantial terminal absence of water-repellence. A rating of 1 or 2 was regarded as satisfactory.

Results are as follows.

| Polyamine |                            | Water Repellence |          |       |      |       |       |
|-----------|----------------------------|------------------|----------|-------|------|-------|-------|
| No.       | Name                       | Glass            | Concrete | Brick | Wood | Cloth | Paper |
| 1         | MBA-ED                     | 2                | 2        | 2     | 2    | 2     | 2     |
| 2         | MBA-TETA                   | 2                | 2        | 2     | 2    | 2     | 2     |
| 3         | MBA-TETA-CH <sub>2</sub> O | 1                | 1        | 2     | 2    | 2     | 2     |
| 4         | PEI                        | 1                | 2        | 2     | 1    | 1     | 1     |
| 5         | IBPA-ED                    | 1                | 1        | 1     | 1    | 1     | 2     |
| 6         | TETA-DCH                   | 2                | 2        | 2     | 2    | 1     | 1     |
| 7         | PVA                        | 1                | 1        | 1     | 2    | 1     | 1     |

The above indicates that best results (Nos. 4, 5 and 7) were to be obtained from high molecular weight linear polyamines largely composed of linkages such as



and



#### Example 8

The following illustrates the application of the method of the present invention to large structural hydrophilic surfaces. For this illustration the substrates selected were two automobile bodies which respectively had baked enamel and nitrocellulose lacquer finishes which had become hydrophilic as the result of several years of weathering.

The bodies were washed with warm soapy water to remove grime and then were thoroughly flushed with fresh water to remove all residual soap. The surfaces were then sponged while wet for five minutes with a 0.5% aqueous solution of polyethylenimine, after which the bodies were again thoroughly flushed with water to remove any unadsorbed polyethylenimine present. While still wet, the bodies were sponged for several minutes with a 0.5% aqueous solution of a commercial soap detergent, having as its active ingredients a mixture of the sodium salts of higher aryl sulfonates and higher alkyl sulfates, after which excess detergent solution flushed off.

When dry, the bodies were highly hydrophobic and shed water as if they had been oiled.

#### Example 9

A porcelain enamel bathtub was thoroughly washed with dilute caustic solution and water and then sponged for a few minutes with a 0.25% aqueous solution of ethylenedichloride-iminobispropylamine condensate. Excess (unadsorbed) amine was then flushed off with fresh

water and the bathtub sponged for a few minutes with a dilute aqueous solution of a commercial hand soap. Excess soap solution was then flushed off. The bathtub became very hydrophobic, and it was noted that its tendency to accumulate scum during use decreased substantially.

I claim:

1. A process of treating a hydrophilic surface to decrease its wettability by water, which comprises contacting said surface with a dilute aqueous solution of a high molecular weight cationic polyamine having an average molecular weight in excess of 10,000 and containing at least one amino nitrogen atom having at least one replaceable hydrogen atom for every 10 carbon atoms therein, thereby irreversibly adsorbing at least some of said polyamine on said surface, and then contacting said surface with sufficient of a dilute aqueous solution of a soap having a hydrophobic anion to convert said adsorbed polyamine to hydrophobic soap form.
2. A process according to claim 1 wherein the surface is concrete.
3. A process according to claim 1 wherein the surface is glass.
4. A process according to claim 1 wherein the surface is a weathered hydrophilic baked pigmented alkyd resin film.
5. A process according to claim 1 wherein the surface is cellulose.
6. A process according to claim 5 wherein the surface is paper.
7. A process according to claim 1 wherein the surface is wood.
8. A process according to claim 1 wherein the polyamine is polyethylenimine.
9. A process according to claim 1 wherein the polyamine is a methylene bisacrylamide-polyalkylenepolyamine condensate.
10. A process according to claim 1 wherein the polyamine is a polyalkylenepolyamine-epichlorohydrin condensate.
11. A process according to claim 1 wherein the surface is contacted with polyamine solution until the adsorptive capacity of the surface for said polyamine is substantially satisfied.
12. A process according to claim 1 wherein after adsorption of the polyamine and before contact of the soap solution the surface is washed with water to remove any unadsorbed polyamine present.
13. A process according to claim 1 wherein the soap having a hydrophobic anion is sodium stearate.
14. A process according to claim 1 wherein the surface is contacted with the dilute aqueous soap solution until formation of polyamine soap has substantially ceased.
15. A process of rendering a surface water-repellent which comprises contacting said surface with an aqueous solution containing 0.01%-1% by weight of a high molecular weight cationic linear chain polyamine having an average molecular weight in excess of 10,000 and containing at least one amino nitrogen atom having at least one replaceable hydrogen atom for every ten carbon atoms therein, until the adsorptive capacity of said surface for said polyamine is substantially satisfied, washing said surface to remove any unadsorbed polyamine present, and then contacting said washed surface with sufficient of a dilute aqueous solution of a soap having a hydrophobic anion to convert said adsorbed polyamine to hydrophobic soap form.
16. A process of rendering a surface water-repellent which comprises contacting said surface with an aqueous neutral solution containing 0.01%-1% by weight of a high molecular weight cationic linear chain polyamine having an average molecular weight in excess of 10,000 and containing at least one amino nitrogen atom having at least one replaceable hydrogen atom for every five

carbon atoms therein, until the adsorptive capacity of said surface for said polyamine is substantially satisfied, washing said surface with water to remove any unadsorbed polyamine present, then contacting said washed surface with sufficient of a dilute aqueous solution of a soap having a hydrophobic anion to convert said adsorbed polyamine to hydrophobic soap form, and drying said surface.

17. A normally hydrophilic surface of decreased wettability by water resulting from the presence thereon in adsorbed form of a polyamine soap formed by interaction of a normally water-soluble polyamine having an average molecular weight in excess of 10,000 and containing at least one amino nitrogen atom having at least one replaceable hydrogen atom for every 10 carbon atoms therein, with a water-soluble soap having a hydrophobic anion.

18. A surface according to claim 17 having adsorbed thereon said adsorbed polyamine soap in amount approximately equivalent to a monomolecular layer.

19. A normally hydrophilic surface rendered water-repellent by the presence thereon of an irreversibly ad-

sorbed small amount of a hydrophobic polyethylenimine stearate, said polyethylenimine stearate containing at least 200 —NHCH<sub>2</sub>CH<sub>2</sub>— units.

5 References Cited in the file of this patent

UNITED STATES PATENTS

|              |                |                |
|--------------|----------------|----------------|
| 2,375,348    | Cohen          | May 8, 1945    |
| 2,495,283    | Werntz         | Jan. 24, 1950  |
| 10 2,573,956 | Daniel et al.  | Nov. 6, 1951   |
| 2,579,033    | Cupery         | Dec. 18, 1951  |
| 2,673,824    | Biefeld et al. | Mar. 30, 1954  |
| 2,677,681    | Gill           | May 4, 1954    |
| 15 2,698,793 | Landes         | Jan. 4, 1955   |
| 2,721,811    | Dacey et al.   | Oct. 25, 1955  |
| 2,729,560    | House et al.   | Jan. 3, 1956   |
| 2,763,571    | Wooding et al. | Sept. 18, 1956 |
| 2,824,861    | Conbere et al. | Feb. 25, 1958  |
| 2,825,714    | Melamed        | Mar. 4, 1958   |
| 20 2,884,057 | Wilson et al.  | Apr. 28, 1959  |
| 2,884,407    | Keim           | Apr. 28, 1959  |